# EUROPEAN PATENT SPECIFICATION

(11) **EP 1 115 562 B1**
(45) Date of publication and mention of the grant of the patent: **31.08.2005**
(21) Application number: 99945214.7
(22) Date of filing: 26.08.1999
(51) Int. Cl.: B32B 5/18, B32B 5/22, C08J 9/30, B32B 5/20

(54) **FOAMED FACER AND INSULATION BOARDS MADE THEREFROM**
GESCHÄUMTE BESCHICHTUNG UND DAMIT HERGESTELLTE ISOLATIONSPLATTEN
BARDAGE EN MOUSSE ET PANNEAUX ISOLANTS QU'IL PERMET DE FABRIQUER

(30) Priority: 08.09.1998 US 99451 P; 18.08.1999 US 376247; 18.08.1999 US 376275
(43) Date of publication of application: 18.07.2001
(73) Proprietor: Building Materials Investment Corporation, Wilmington, DE 19801 (US)
(72) Inventor: HORNER, Charles, J., Jr., Piscataway, NJ 08854 (US); FRANZYSHEN, Frank, S., South Bound Brook, NJ 08880 (US); SHERMAN, Murray, S., Leland, NC 28451 (US)
(74) Representative: Harrison, David Christopher
(86) International application number: PCT/US1999/019499
(87) International publication number: WO 2000/014358

(56) References cited:
- US-A- 5 001 005
- US-A- 5 102 728
- US-A- 5 717 012

## Description

### BACKGROUND OF THE INVENTION

Rigid polymeric foam insulation laminates have been used for many years by the construction industry. Uses include commercial roof insulation boards utilized under asphaltic built-up roof (BUR) membranes as well as under various single ply membranes such as EPDM rubber, PVC, modified bitumen membranes and the like. Other uses include residential insulation, as sheathing under siding, and as roof insulation under asphalt shingles and concrete tiles.

Such insulation often takes the form of a core polymeric foamed thermoset material such as polyurethane, polyisocyanurate, polyurethane modified polyisocyanurate (often referred to as polyiso) or phenolic resin, applied between two facing sheets.

These insulation boards are generally manufactured on production lines where a liquid core chemical mixture is poured over a bottom facer, foaming up to contact a top facer in a constrained rise laminator. The reaction of the chemical mixture causing foaming is generally exothermic, as curing via polymerization and crosslinking occurs in the laminator. In the case of polyisocyanurate insulation boards, the curing exotherm lasts well into the time the resulting rigid boards are cut, stacked and warehoused. The exotherm can continue for as long as 4 days and the mixture can reach temperatures as high as 163°C (325°F).

Desirable properties for the facers include flexibility, high tensile and tear strength and resistance to thermal degradation. Facer porosity should be low and the thickness of the facer coating should be sufficient to prevent bleed-through of the liquid chemicals prior to foaming. Additionally, facers should exhibit good adhesion to the core foam insulation and be inert to the effects of extraneous chemicals which may be present in the mixture, especially blowing agents that also behave as solvents. Blowing agents currently in use include chlorofluorocarbons like HCFC-141b and R-22 as well as hydrocarbons such as n-pentane, cyclo-pentane and iso-pentane.

One problem that has plagued the polyiso industry has been a phenomenon called "cold temperature delamination". This phenomenon occurs in cold temperature areas where insulation boards coming off the production line cool before they can be "stack cured". In a worst case scenario, the polyiso core foam layer closest to the facer cools, quenching the cure reaction and leaving a brittle layer. This often leads to shearing of the core layer or facer peal off. It has been the practice of manufacturers to place a layer of corrugated cardboard over both the top facer surface of the top board and under the bottom facer surface of the bottom board in the stack, to retain exothermic heat and prevent subsequent delamination. Thus, a facer that inherently insulates and retains heat during stack cure would materially reduce incidents of cold temperature delamination and would eliminate the need for costly cardboard insulation.

After these foamed polymer insulation boards are cured, cut and shipped to their use site, the facer should provide mechanical stability as well as water and weather resistance since, upon installation, they may be exposed to persistent rain, high humidity, ultraviolet light and excessive heat. Additionally, the facers must be puncture and scuff resistant to survive being nailed and walked on. Withstanding temperatures up to 260°C (500°F), as encountered in hot asphalt applications, as well as resistance to the deleterious effects of adhesive solvents used in single ply roofing membrane applications while strongly bonding to the adhesives themselves are also important facer properties.

Traditionally, facer materials have included asphalt saturated cellulosic felts, fiberglass mats, asphalt emulsion coated fiberglass mats, aluminum foil/Kraft/foil, glass fiber modified cellulosic felts, glass mats onto which polymeric films have been extruded, and glass mats coated with polymeric latex/inorganic binder coatings. However, all of these materials have at least one undesirable property. For example, asphalt-containing products are not compatible with PVC single ply roofing membranes. Fiberglass mats are subject to excessive bleed-through of foamable core chemicals. Aluminum facers and foils reflect heat into the foam during processing which leads to disruption of cell structure, delamination and warping. Further, foil faced sheathing and extrusion or lamination of a polymer film to glass mat surfaces are costly. Specifically, glass mats coated with polymer latex/inorganic binder mixtures have been found to be brittle; conversely, glass fiber modified cellulosic felts are susceptible to moisture absorption aggravating board warping in damp or wet environments.

Other facers which have been employed for siding underlayment and insulation board facers include those disclosed in U.S. Patents 5,776,841 and 5,717,012, which are primarily felts.

U.S. Patent No. 5,001,005 describes a facing sheet composed of glass fibers and a non-asphaltic binder. The facer contains 60-90% glass fibers, which high fiber content does not provide sufficient binder to close the sheet's pores or to provide desired sheet strength. U.S. Patent No. 5,102,728, describing a glass mat substrate coated with a polymeric latex blended with an asphalt emulsion, concerns a product which is not only incompatible with PVC roofing membranes but also requires excessive coating thicknesses to reduce high porosity. Accordingly, this product is very costly. U.S. Patent No. 5,112,678 discloses a facer prepared by applying to a fiberglass mat a flowable polymer latex and an inorganic binder coating. The resulting product is somewhat brittle and is susceptible to an undesirable degree of chemical bleed through. U.S. Patent Nos. 5,698,302 and 5,698,304 describe facers where polymer films are laminated or extruded onto fiberglass mat. Not only is this approach costly, but also since conventional mineral flame retardant filled polymers do not extrude well, some degree of resistance to flammability must be sacrificed.

Accordingly it is an object of this invention to overcome the above disadvantages and deficiencies and to provide a facer which is economically produced by a commercially feasible process.

It is also an object to provide a mechanically stable facer suitable for insulation board manufacture which resists cold temperature delamination and which has superior tolerance to the effects of weathering.

Another object is to provide a facer which exhibits superior adhesion to polyiso foam of an insulation board core material.

These and other objects and advantages of the invention will become apparent from the following description and disclosure.

### SUMMARY OF THE INVENTION

The non-asphaltic, non-cellulosic facer of the present invention comprises a dry, preformed fibrous mat substrate on which is coated a pre-frothed or pre-foamed composition containing a natural or synthetic thixotropic latex polymer, a surfactant and an inorganic mineral filler. The composition may optionally contain up to about 15 wt.% of extraneous additives, which include a flame retardant, dye, thickener, porosity reducing agent, thermal and/or UV stabilizers and the like, to provide a foamed facer product having, on a dry weight basis, less than 50% fiber in the mat. The preferred facer product contains 30 to 46. wt.% of fiber in the composition consisting of mat fiber with binder and latex in the coating mixture.

### DETAILED DESCRIPTION OF THE INVENTION

Generally, the foamed coating composition applied to the preformed mat contains on a dry weight basis between 15 and 80 wt.% of the thixotropic polymer latex, between 0.01 and 80 wt.% filler, between 0.5 and 10 wt.% foam supporting surfactant and 0 to 15 wt.% extraneous additives.

The fibers of the mat employed in this invention include any of the non-cellulosic types, such as fibers of glass, polyester, polypropylene, polyester/polyethylene/teraphthalate copolymers, hybrid types such as polyethylene/glass fibers and other conventional non-cellulosic fibers. Mats having glass fibers in random orientation are preferred for their resistance to heat generated during the manufacture of insulation boards and flame resistance in the finished product.

The fibrous mats of the invention, generally of between 254 and 762 x 10⁻³ mm (10 and 30 mils) thickness, conventionally contain a binder which is incorporated during mat formation to fix the fibers in a self-sustaining solid web and to prevent loss of fibers during subsequent processing and handling. Such binders include phenol-, melamine- and/or urea- formaldehyde resins or mixtures thereof. Most preferred are the mats having glass fibers in the range of from 3 to 20 microns, most desirably 10-18 microns, in diameter and a length of from 0.64 cm to 4.45 cm (0.25 to 1.75 inch), most desirably a length of 1.91 to 3.81 cm (0.75-1.5 inch).

The fillers useful in the present coating mixture include conventional inorganic types such as clays, mica, talc, limestone, kaolin, other stone dusts, gypsum, aluminum silicate (e.g. Ecca Tex 561), flame retardant aluminum trihydrate, ammonium sulfamate, antimony oxide, calcium silicate, calcium sulfate, and mixtures thereof.

Surfactants employed in the coating composition are organic types suitable for stabilizing latices, such as for example, ammonium salts of a C₁₀ to C₂₂ fatty acid, e.g. ammonium stearate (STANFAX 320). One or more surfactants can be employed in the coating composition to promote the formation of foam and to maintain the foam structure of the coating before curing.

The latex component of the coating composition includes latex polymers of natural rubber as well as synthetic latices including copolymers of styrene and butadiene and acrylic based resins. Representative examples of these are polyvinyl chloride, styrene/acrylic or methacrylic esters, ethylene/vinyl chloride and polyurethane, polyisoprene, polyvinylidene chloride, polyvinyl acetate/polyvinyl chloride and synthetic rubbers such as SBS, SBR, neoprene, etc. and any other thixotropic latex polymer and mixtures of the foregoing.

The mat coating mixture of the invention is obtained from a frothed or foamed 15-80 wt.% aqueous emulsion, dispersion or suspension, which is prefoamed by incorporating air in the aqueous liquid mixture, e.g. by blowing or mixing, with vigorous agitation in the presence or absence of a conventional blowing agent. The resulting frothed or foamed, aerated composition is then coated to a thickness of from 127 to 2540 x 10⁻³ mm (5 to 100 mils) on the preformed mat surface under ambient conditions using a knife blade, a roller or any other convenient method of application. In one aspect, the foam coated mat is then dried at below its cure temperature to provide a foamed, self-supporting product having a reduced coating thickness of up to 2286 x 10⁻³ mm (90 mils) which adheres to the mat surface. In another aspect, the foamed coated mat is dried and cured simultaneously.

The resulting facer product of this invention is desirably flexible and possesses low permability to liquid chemicals used for insulation cores as well as superior dimensional stability and high tensile strength after curing. This product, comprising the mat having an adhered surface coating of a prefoamed latex/filler/surfactant, can be fed directly to insulation board manufacture, e.g. a constricted rise laminator, wherein the uncoated fiber surface of the mat contacts at least one exposed surface of a foamed or foamable thermosetting non-elastomeric core in the manufacture of an insulation board as described hereinafter.

As indicated above, the foamed coating of the present facer can be formed in the absence or presence of a blowing agent to provide a composition of reduced density, which density can be reduced from above about 2 g/cm³ (g/cc) to as little as 0.15 g/cm³ (g/cc). Advantageously, the consistency of the foam is such that the coating mixture does not penetrate through the mat and ideally simulates the consistency of shaving cream.

Generally the amount of air incorporated into the foamable mixture prior to coating is between about 5% and about 80% by volume for optimal consistency and the resulting foamed mixture has bubble openings sufficiently small so as to inhibit liquid bleed through the mat.

Applying a film or laminating a layer of impervious resin or polymer over the foamed surface to provide a trilayered facer member can provide a totally liquid impervious surface on the facer, in special cases where such is desired. A top seal coat of a non-foamed latex is suitable for this purpose. Alternatively, a thermoplastic such as polyethylene powder or unexpanded polystyrene beads can be used as a filler which melts at the drying/curing temperatures to close substantially all pores of the pervious coating. Expandable excipients and additives such as cellulose can also be used for this purpose; although the use of a seal coat is neither needed nor recommended. Other methods for accomplishing the similar purpose include the use of less air during foaming, the omission or use of less inorganic filler in the coating composition, calendering and/or embossing the foamed or frothed surface by contact with a hot roller or platen. Still another method for producing the totally impervious surface involves forming the foam on the smooth surface of a conventional release material and then contacting the mat with the opposite surface of the foam. A combination of any of the above options can be employed for specialized purposes if desired.

In the present case, the facer of the invention having a foamed cellular coating, contains latent exothermic energy and has a higher potential heat capacity upon entering the laminator; thus lowering the lamination cure time and prolonging the generation of heat by acting as an insulator during curing in the post cure stack. This advantage eliminates the need for heat retaining members at the top and bottom of the stack and significantly reduces the prior problem of the board's susceptibility to cold temperature delamination. Additionally, where the foamed coating on the facer is dried and/or cured, the bonding strength between the uncoated fibers and the core material in the resulting product is enhanced due to reduced penetration of the coating mixture into the mat by reason of its prefoamed state. Where the foam of the facer is completely cured before entering the laminator, the core material is cither poured onto the uncoated fibrous surface of the facer or laminated thereto with adhesive or bonding agent.

Any pressure which may be applied during lamination in the insulation board manufacture is less than that required to cause a 50% reduction in the thickness of the foamed facer coating and insufficient to result in damage or crushing of the mat fibers in the finished insulation board product.

The weight of the present facer can vary from 40 to 300 g/sq. meter and the foamed facer sheet can have a thickness up to 2540 x 10⁻³ mm (100 mils) depending on the preference of the consumer. For certain purposes demanding tougher facers, laticies which can be crosslinked can be selected.

The present latex coating composition may additionally contain a minor amount, up to 15%, preferably less than about 3 wt.%, of a conventional thickening agent, for example an acrylic polymer thickener, e.g. (ACRYSOL ASE 95NP and/or 60NP) and the like. Other inert excipients such as a UV or thermal stabilizer, a conventional coloring agent, texturizing agent, reinforcing or crosslinking agent, (e.g. CYMEL 303 resin) and/or blowing agent may also be included in the coating mixture; although addition of these additives in a minor amount of less than 2 wt.% are preferred.

The insulation boards, for which the present facer is particularly suited, comprise conventional thermosetting or thermoplastic foam cores, such as foamed polyurethane or polyurethane modified polyisocyanurate or phenol-formaldehyde cores disposed between a pair of facer members which are laminated to the core surfaces. Other non-elastomeric foamable chemicals, such as polyvinyl chloride, polystyrene, polyethylene, polypropylene, and others conventionally employed as core material can also be employed as the insulation board core of this invention. Rigid foamed cores of this type are described for example in U. S. Patent 4,351,873.

The present facers are also suitable for sheathing a siding underlayment generally of a thickness up to about 2.54 cm (1 inch) and composed of a non-elastic core material of a chemical or chemical mixture similar to that of the insulation core. The use of instant facer eliminates the need for expensive foil facings which hold and reflect heat and often cause warping and deterioration of wood overlayment. Also, foil and similar facings are easily punctured which gives rise to moisture attack.

In the insulation manufacture, a roll of the present foamed facer sheet product is passed, with its uncoated fiber surface opposite the core surface, to a laminating zone. The board core foam precursor chemical or mixture of chemicals can be poured onto the non-coated fiber surface of the facer sheet or the core of the insulation board can be prefoamed to a self-sustaining consistency. In one embodiment, a first facer of this invention, with its uncoated surface abutting the core, is placed below the core. The fiber surface of a second facer is positioned and spaced above the core to allow for core expansion, e.g. in a constricted rise laminator, where the assembly undergoes an exothermic reaction and curing is initiated. During the curing operation the core material foams and rises to engage the lower uncoated surface of the second facer. It is to be understood that one of the first and second facers can be of the same or of a different composition than that of this invention; although it is preferred that both of these facers be those of the invention described herein. More specifically, one of the facer sheets may be selected from those conventionally employed, such as for example a cellulose or cellulose-glass hybrid felt sheet, perlite, aluminum foil, multilaminated sheets of foil and Kraft, uncoated or coated fiber glass mats; although the second facer sheet of the present invention enhances the advantages described herein. As the core foam is spread on the fibrous surface of the first facer sheet entering the laminator, it undergoes an exothermic reaction which can attain a temperature up to about 93°C (200°F). The core foam rises to contact the undersurface of the second facer and hardens thereon; thus providing a rigid insulating foam core interposed or sandwiched between two facer sheets. The resulting product can then be cut into boards of desired size and shape. The heat of the exothermic reaction involving polymerization and/or crosslinking, is autogenerated in both the laminator and in the subsequent stacking of insulation boards to insure complete curing of the core and surface coating of the facer. Curing temperatures during stacking can rise up to about 163°C (325°F) over a period of up to 4 days.

As another embodiment involving the above operation, the top and bottom positioning of the facer sheets can be reversed so that the facer of this invention is fed and spaced above a conventional facer in a manner such that its non-coated fibrous surface faces the foamable insulating core chemical being contacted on its under surface with another facer sheet. The later procedure is practiced where one facer is a rigid sheet, as in a perlite or particle board facer as opposed to the flexible facer of this invention which can be fed to the laminator as a continuous roll. In this case the foamable insulating core chemical is surfaced on the rigid facer member and rises to engage the fibrous uncoated surface of the present facer.

The latex of the present facer surface layer which, due to its comparatively thick latex foam, and low fiber to coating latex ratio, more efficiently retains heat between the layers of the roll. Hence, lamination of the core can be completed at a faster rate and stacking accomplished without damage to the laminate. Additionally, it is now found that this retention of heat during curing improves core bonding and significantly reduces subsequent "cold temperature delamination" in the product, which is caused by failure of the top layer of insulation to completely cure due to cooler temperature exposure during stacking after leaving the laminator.

The insulation boards incorporating the present facers are useful in commercial roof insulation, residential or commercial wall sheathing etc. Depending upon the intended use, the present insulation board has a core thickness which may vary widely, for example between 1.27 and 10.2 cm (0.5 and 4 inches) or more.

In the above discussion, it will become apparent that it is also possible to form the insulation core separately, i.e. absent contact with the fibers of a facer, and subsequently bond one or more of the present facers to the core using suitable adhesives. In general, the teachings of U.S. Patent 4,351,873 are applicable to the formation of rigid foam cores and adhesion of facer sheets to at least one surface of such cores.

Polyurethane or polyisocyanurate are most commonly employed as core materials; although other non-elastomeric, foamable chemicals are also employed. Examples of the later include polyvinyl chloride, polystyrene, phenolic resins and the like.

The facers and the insulation board products of this invention exhibit significantly higher tensile strength than those containing 60-90 wt.% fibers. The present facers also possess resistance to cracking at low temperatures and exceptionally superior dimensional stability and flame retardance. Because of their superior strength and flexibility, the present facer can find broader application, such as non-foil, non-glare sheathings, as shingle underlayment, separation or barrier sheets and the like.

### EXAMPLE 1

A 473 ml metal can with a low shear mixer was employed to combine a 51.5 % aqueous solution of a self crosslinkable acrylic latex (Rohm & Haas, E-693), a 23.5% aqueous clay slurry (Ecca Tex 561), a mixture of a melamine crosslinking agent (CYMEL 303), an ammonium stearate foam stabilizer (STANFAX 320), an acrylic polymer thickening agent (Acrysol ASE 95NP) and carbon black pigment in amounts shown in following Table 1. The above ingredients were thoroughly mixed for about 10 minutes and then foamed using a high speed Kitchen Aid mixer to produce a foam having a density of 0.2 (g./cc) g/cm³. The Brookfield viscosity of the foamed mixture, using an LVT #4 spindle at 30 rpm, was 1,500 cps.

**TABLE 1**

| INGREDIENT | % Solids | Parts Wet Basis | Parts Dry Basis |
|---|---|---|---|
| Acrylic latex | 48.5 | 100 | 48.50 |
| Kaolin slurry | 76.5 | 90 | 68.85 |
| CYMEL 303 | 100 | 1.5 | 1.50 |
| STANFAX 320* | 33 | 8.0 | 2.64 |
| Acrysol ASE 95NP | | | |
| Water (1/1 mole) | 9.3 | 0.8 | 0.07 |
| Carbon black | 33 | 0.45 | 0.15 |

| | | | |
|---|---|---|---|
| * ammonium stearate | | | |

The above foamed latex mixture was coated onto the upper surface of a preformed glass fiber mat containing 27.5 wt.% urea-formaldehyde binder and having 72.5 wt.% of average 3.18 cm (1¼ inch) long filaments of 15.9 micron average diameter. Coating was accomplished using a Gardner draw-down gauge set to achieve a coating thickness of 762 x 10⁻³ mm (30 mils) on the mat. The resulting sample was dried in an oven at 125°C. for 3 minutes and then cured at 150°C. for an additional 3 minutes.

The properties of above facer sample was compared with those of commercial samples A, B and C. and the results were as recorded in Table 2.

### EXAMPLE 2

Example 1 was repeated except that self-crosslinkable acrylic (RHOPLEX B-959) was substituted for latex (E-693) and the dried prefoamed mixture on the mat was not cured. The unfoamed mixture of this example had a Brookfield viscosity of 3,600 cps.

The uncured, foam-coated mat of this example was introduced to a laminator wherein the uncoated fiber under surface of the mat was contacted with a foamed polyurethane/isocyanurate core of an insulation board and the simultaneous curing of the mat foam and the core was initiated. After about 1-2 minutes in the laminator, at a temperature of about 120° to 200°C, the laminated board was cut into 122 x 244 cm (4 x 8 foot) boards and the boards squares stacked in units of 25 members to complete curing over a period of 2.5 days.

### EXAMPLE 3

Example 1 was repeated except that an additional 45 g of aluminum trihydrate (ALCOA GRADE C-320) was added to the coating mixture to increase flame retardance of the facer. The Brookfield viscosity of the unfoamed mixture was 2,200 cps and the foam had a density of 0.23 (g/cc) g/cm³.

Conventional facers most commonly employed are non-coated, cellulose fiber mats which may or may not be reinforced with a minor amount of glass fibers. In Table 2, Examples A and B represent this type. Example A is reinforced with 18% of 3.2 cm (1¼ inch) long glass fibers, Example B is reinforced with 13% of less than 0.32 cm (1/8 inch) long glass fibers.

Another type of facer which has had commercial success comprises a glass mat on which a polyethylene coating has been extruded. A facer of this type is represented as Sample C.

The properties of all of the facers in the above examples are reported in following Table 2.

The above examples are representative and it will be understood that many alterations and substitutions can be made therein without departing from the scope of this invention. Reference defining the invention is had to the appended claims.

## Claims

1. A flexible, low fiber containing facer suitable for use in building construction and containing on a dry weight basis less than 50 wt.% fiber, which comprises a non-asphaltic, non-cellulosic fiber mat substrate of between 254 and 762 x 10⁻³ mm (10 and 30 mils) thickness, which mat substrate is in contact with a 127 to 2540 x 10⁻³ mm (5 to 100 mil) thick mat surface coating, said coating being obtained from a foamed 15-80 wt.% aqueous mixture containing, on a dry weight basis, (a) between 15 and 80 wt.% of a thixotropix polymer latex, (b) between 0.01 and 80 wt.% of inorganic filler and (c) between 0.5 and 10 wt.% of an organic surfactant.

2. The facer of claim 1 wherein the fiber of said mat is glass fiber.

3. The facer of claim 2 wherein said fibers have an average diameter between about 3 and about 20 microns and a length of between 0.64 and 4.5 cm (0.25 and 1.75 inch).

4. The facer of claim 1 wherein (c) is an ammonium salt of a C₁₀ to C₂₂ fatty acid.

5. The facer of claim 6 wherein (c) is ammonium stearate.

6. The facer of claim 1 wherein said latex of the coating mixture is an acrylic based resin.

7. The facer of claim 1 wherein said coating mixture additionally contains up to 15 wt.% of an excipient selected from the group of a thickener, a coloring agent, a texturizing agent, a UV light stabilizer, a thermal stabilizer, a flame retardant, a weather resistance agent and a blowing agent.

8. The facer of claim 7 wherein a UV stabilizer is present in an amount up to about 2.5 wt.% of the mixture.

9. The facer of claim 1 wherein the facer contains 30 to 46 wt.% of fiber.

10. The facer of claim 1 wherein said coating has a density of between about 0.1 and about 4 g/cm³ (g./cc).

11. The process for preparing the facer of claim 1 which comprises:
(a) forming a 15 to 80 wt.% aqueous mixture of said coating composition,
(b) foaming said mixture to a self-sustaining consistency,
(c) applying a 127 to 2032 x 10⁻³ mm (5 to 80 mil) uniform coating of the foamed mixture to one surface of said mat,
(d) drying the resulting mat and
(e) recovering the dried, foam coated mat having a fiber concentration below 50 wt.% as the product of the process.

12. The process of claim 11 wherein the foam coated facer is dried and cured and then passed to a laminator for lamination to a non-elastic insulation board core.

13. The process of claim 11 wherein the foam coated facer is dried at below its curing temperature and is then passed to a laminator where the dried foam is contacted with a non-elastic lamination board core and is cured thereon.

14. A siding underlayment having a conventional non-elastic core laminated to a facer of claim 1.

15. An insulation board having a non-elastic core laminated on a surface to a low fiber containing, non-asphaltic and non-cellulosic mat of claim 1.

16. The insulation board of claim 15 wherein said surfactant is an ammonium salt of a C₁₀ to C₂₂ fatty acid.

17. The insulation board of claim 16 wherein said salt is ammonium stearate.

18. The insulation board of claim 15 having a non-elastic core wherein both surfaces of said core are laminated to a facer of claim 1.

19. The insulation board of claim 15 having a non-elastic core wherein one surface of the core is laminated to the facer of claim 1.

20. The insulation board of claim 19 wherein the opposite surface of said core is laminated to a conventional cellulose- or asphaltic- containing mat.

21. The insulation board of claim 15 wherein the latex of said latex is an acrylic based resin.

22. The insulation board of claim 15 wherein said filler is a fire retardant agent.

23. The insulation board of claim 22 wherein said filler is aluminum trihydrate.

24. The insulation board of claim 15 wherein said mat contains less than 50 wt.% fiber.

25. The insulation board of claim 24 wherein said mat contains between 30 and 46 wt.% fiber.

26. The insulation board of claim 15 wherein said facer is a glass mat surfaced with said cured foam.

27. The insulation board of claim 15 having a thickness of between 0.5 and 10.2 cm (0.2 and 4 inches).

28. The insulation board of claim 15 wherein said cured foam has a density of between 0.1 and 0.4 g/cm³ (g./cc).

## Revendications

1. Un barbage souple contenant une faible proportion de fibres, approprié pour être utilisé dans la construction immobilière et contenant, sur une base de poids sec, moins de 50% en poids de fibres, lequel comprend un substrat de matelas de fibres non-asphaltiques et non-cellulosiques d'entre 254 et 762 x 10⁻³ mm (10 et 30 mils) d'épaisseur, lequel substrat de matelas est en contact avec un revêtement de surface de matelas épais (5 à 100 mils) 127 à 2540 x 10⁻³ mm, ledit revêtement étant obtenu à partir d'un mélange aqueux en mousse de 15 à 80% en poids contenant, sur une base de poids sec, (a) entre 15 et 80% en poids d'un latex de polymère thixotrope, (b) entre 0,01 et 80% en poids d'une charge minérale et (c) entre 0,5 et 10% en poids d'un tensioactif organique.

2. Le bardage de la revendication 1 dans lequel la fibre dudit matelas est de la fibre de verre.

3. Le bardage de la revendication 2 dans lequel lesdites fibres ont un diamètre moyen entre environ 3 et environ 20 microns et une longueur d'entre 0,64 et 4,5 cm (0,25 et 1,75 pouces).

4. Le bardage de la revendication 1 dans lequel (c) est un sel d'ammonium d'un acide gras en C₁₀ à C₂₂.

5. Le bardage de la revendication 6 dans lequel (c) est du stéarate d'ammonium.

6. Le bardage de la revendication 1 dans lequel ledit latex du mélange de revêtement est une résine à base acrylique.

7. Le bardage de la revendication 1 dans lequel ledit mélange de revêtement contient en outre jusqu'à 15% en poids d'un excipient sélectionné dans le groupe d'un épaississeur, d'un agent colorant, d'un agent de texturation, d'un stabilisant contre l'effet de la lumière ultraviolette, d'un stabilisant thermique, d'un ignifuge, d'un agent de résistance aux intempéries et d'un agent de moussage.

8. Le bardage de la revendication 7 dans lequel le stabilisant contre l'effet des ultraviolets est présent dans une quantité allant jusqu'à 2,5% en poids du mélange.

9. Le bardage de la revendication 1 dans lequel le bardage contient 30 à 46% en poids de fibres.

10. Le bardage de la revendication 1 dans lequel ledit revêtement a une densité d'entre environ 0,1 et environ 4 g/cm³ (g./cc).

11. Le procédé de fabrication du bardage de la revendication 1 qui comprend les étapes consistant à:
(a) former un mélange aqueux de 15 à 80% en poids de ladite composition de revêtement,
(b) faire mousser ledit mélange à une consistance auto-sustentatrice,
(c) appliquer un revêtement uniforme de 127 à 2032 x 10⁻³ mm (5 à 80 mils) du mélange en mousse sur une surface dudit matelas,
(d) sécher le matelas résultant et
(e) récupérer le matelas séché, revêtu de mousse et présentant une concentration en fibres en dessous de 50% en poids, comme étant le produit du procédé.

12. Le procédé de la revendication 11 dans lequel le bardage revêtu de mousse est séché et amené à polymériser et est amené ensuite à passer vers une machine à stratifier en vue d'une stratification sur un noyau de panneau isolant non élastique.

13. Le procédé de la revendication 11 dans lequel le bardage revêtu de mousse est séché à en dessous de sa température de polymérisation et est ensuite amené à passer vers une machine à stratifier où la mousse séchée est mise en contact avec un noyau de panneau de stratification non élastique et est polymérisé sur lui.

14. Une sous-couche de mise de côté comprenant un noyau non-élastique de type traditionnel stratifié sur un bardage de la revendication 1.

15. Un panneau isolant comprenant un noyau non élastique stratifié sur une surface d'un matelas non asphaltique et non-cellulosique contenant une faible proportion de fibres selon la revendication 1.

16. Le panneau isolant de la revendication 15 dans lequel ledit tensioactif est un sel d'ammonium d'un acide gras en C₁₀ à C₂₂.

17. Le panneau isolant de la revendication 16 dans lequel ledit sel est du stéarate d'ammonium.

18. Le panneau isolant de la revendication 15 comprenant un noyau non élastique dans lequel les deux surfaces du noyau sont stratifiées sur un bardage de la revendication 1.

19. Le panneau isolant de la revendication 15 comprenant un noyau non élastique dans lequel une surface du noyau est stratifiée sur le bardage de la revendication 1.

20. Le panneau isolant de la revendication 19 dans lequel la surface opposée dudit noyau est stratifiée sur un matelas à contenance cellulosique ou asphaltique de type traditionnel.

21. Le panneau isolant de la revendication 15 dans lequel le latex dudit latex est une résine à base acrylique.

22. Le panneau isolant de la revendication 15 dans lequel ladite charge est un agent ignifuge.

23. Le panneau isolant de la revendication 22 dans lequel ladite charge est de l'aluminium trihydraté.

24. Le panneau isolant de la revendication 15 dans lequel ledit matelas contient moins de 50% en poids de fibres.

25. Le panneau isolant de la revendication 24 dans lequel ledit matelas contient entre environ 30 et 46% en poids de fibres.

26. Le panneau isolant de la revendication 15 dans lequel ledit bardage est un matelas de verre avec ladite mousse polymérisée en surface.

27. Le panneau isolant de la revendication 15 présentant une épaisseur d'entre 0,5 et 10,2 cm (0,2 et 4 pouces).

28. Le panneau isolant de la revendication 15 dans lequel ladite mousse polymérisée a une densité d'entre 0,1 et 0,4 g/cm³ (g./cc).

## Patentansprüche

1. Flexible Abdeckung mit geringem Fasergehalt, die zur Verwendung im Hochbau geeignet ist und, bezogen auf das Trockengewicht, weniger als 50 Gew.-% Fasern enthält, umfassend ein asphaltfreies, cellulosefreies Fasermattensubstrat mit einer Dicke zwischen 254 und 762 x 10⁻³ mm (10 und 30 Mil), wobei das Mattensubstrat in Kontakt mit einer 127 bis 2540 x 10⁻³ mm (5 bis 100 Mil) dicken Mattenoberflächenbeschichtung ist, wobei die Beschichtung aus einem geschäumten 15-80 gewichtsprozentigen wässrigen Gemisch erhalten wird, das, bezogen auf das Trockengewicht, (a) zwischen 15 und 80 Gew.-% eines thixotropen Polymerlatex, (b) zwischen 0,01 und 80 Gew.-% eines anorganischen Füllstoffs und (c) zwischen 0,5 und 10 Gew.-% eines organischen Tensids enthält.

2. Abdeckung nach Anspruch 1, worin die Fasern der Matte Glasfasern sind.

3. Abdeckung nach Anspruch 2, worin die Fasern einen mittleren Durchmesser zwischen etwa 3 und etwa 20 µm und eine Länge von zwischen 0,64 und 4,5 cm (0,25 und 1,75 Zoll) aufweisen.

4. Abdeckung nach Anspruch 1, worin (c) ein Ammoniumsalz einer C₁₀- bis C₂₂-Fettsäure ist.

5. Abdeckung nach Anspruch 6, worin (c) Ammoniumstearat ist.

6. Abdeckung nach Anspruch 1, worin der Latex des Beschichtungsgemischs ein Harz auf Acrylbasis ist.

7. Abdeckung nach Anspruch 1, worin das Beschichtungsgemisch außerdem bis zu 15 Gew.-% eines Hilfsstoffs umfasst, der aus der aus einem Verdickungsmittel, einem Farbstoff, einem Texturierungsmittel, einem UV-Lichtstabilisator, einem Wärmestabilisator, einem Flammverzögerungsmittel, einem Witterungsbeständigkeitsmittel und einem Treibmittel bestehenden Gruppe ausgewählt ist.

8. Abdeckung nach Anspruch 7, worin ein UV-Stabilisator in einer Menge von bis zu 2,5 Gew.-% des Gemischs vorhanden ist.

9. Abdeckung nach Anspruch 1, worin die Abdeckung 30 bis 46 Gew.-% Fasern enthält.

10. Abdeckung nach Anspruch 1, worin die Beschichtung eine Dichte von zwischen etwa 0,1 und etwa 4 g/cm³ aufweist.

11. Verfahren zur Herstellung einer Abdeckung nach Anspruch 1, umfassend:
(a) das Bilden eines 15-80 gewichtsprozentigen wässrigen Gemischs aus der Beschichtungszusammensetzung,
(b) das Schäumen des Gemischs auf eine selbsterhaltende Konsistenz,
(c) das Auftragen einer 127 bis 2032 x 10⁻³ mm (5 bis 80 Mil) dicken gleichmäßigen Beschichtung aus dem geschäumten Gemisch auf eine Oberfläche der Matte,
(d) das Trocknen der resultierenden Matte und
(e) das Erhalten der getrockneten, schaumbeschichteten Matte mit einer Faserkonzentration unter 50 Gew.-% als Produkt des Verfahrens.

12. Verfahren nach Anspruch 11, worin die schaumbeschichtete Abdeckung getrocknet und gehärtet und dann in eine Laminiermaschine gegeben wird, um sie an einen nichtelastischen Dämmplattenkern zu laminieren.

13. Verfahren nach Anspruch 11, worin die schaumbeschichtete Abdeckung bei einer Temperatur unter ihrer Härtungstemperatur getrocknet und dann in eine Laminiermaschine gegeben wird, wo der getrocknete Schaum mit einem nichtelastischen Laminatplattenkern in Kontakt gebracht und darauf gehärtet wird.

14. Außenverkleidungsunterlage mit einem herkömmlichen nichtelastischen Kern, der auf eine Abdeckung nach Anspruch 1 laminiert ist.

15. Dämmplatte mit einem nichtelastischen Kern, die mit einer Oberfläche auf eine asphaltfreie, cellulosefreie Matte mit geringem Fasergehalt nach Anspruch 1 laminiert ist.

16. Dämmplatte nach Anspruch 15, worin das Tensid ein Ammoniumsalz einer C₁₀-bis C₂₂-Fettsäure ist.

17. Dämmplatte nach Anspruch 16, worin das Salz Ammoniumstearat ist.

18. Dämmplatte nach Anspruch 15 mit einem nichtelastischen Kern, worin beide Oberflächen des Kerns auf eine Abdeckung nach Anspruch 1 laminiert sind.

19. Dämmplatte nach Anspruch 15 mit einem nichtelastischen Kern, worin eine Oberfläche des Kerns auf eine Abdeckung nach Anspruch 1 laminiert ist.

20. Dämmplatte nach Anspruch 19, worin die gegenüber liegende Oberfläche des Kerns auf eine herkömmliche cellulose- oder asphalthältige Matte laminiert ist.

21. Dämmplatte nach Anspruch 15, worin der Latex des Latex ein Harz auf Acrylbasis ist.

22. Dämmplatte nach Anspruch 15, worin der Füllstoff ein flammhemmendes Mittel ist.

23. Dämmplatte nach Anspruch 22, worin der Füllstoff Aluminiumtrihydrat ist.

24. Dämmplatte nach Anspruch 15, worin die Matte weniger als 50 Gew.-% Fasern enthält.

25. Dämmplatte nach Anspruch 24, worin die Matte zwischen 30 und 46 Gew.-% Fasern enthält.

26. Dämmplatte nach Anspruch 15, worin die Abdeckplatte eine Glasmatte ist, die mit dem gehärteten Schaum beschichtet ist.

27. Dämmplatte nach Anspruch 15 mit einer Dicke zwischen 0,5 und 10,2 cm (0,2 und 4 Zoll).

28. Dämmplatte nach Anspruch 15, worin der gehärtete Schaum eine Dichte zwischen 0,1 und 0,4 g/cm³ aufweist.
